

## UNITED STATES PATENT OFFICE

2,091,633

SANITARY FOOD CONTAINER AND METHOD  
OF MAKINGMark W. Frishkorn, Cincinnati, Ohio, assignor to  
The International Printing Ink Corporation,  
New York, N. Y., a corporation of OhioNo Drawing. Application August 7, 1935,  
Serial No. 35,065

4 Claims. (Cl. 99—181)

This invention relates to food containers and aims to provide metal containers which will keep foodstuffs of all sorts free from contamination of taste and the interior surface of the container 5 free from contamination of color.

The object of this invention is to provide a standard lining for alkaline foodstuff containers, including particularly those used for asparagus and spinach.

10 It has heretofore been customary to provide metal food containers such as tin cans with a lining consisting of an oleoresinous film with a moderate proportion of zinc oxide varying from 3½ to 5%. It has been found that such linings 15 permit two-way reactions between the food and the metal, which result in contaminating the taste of the food. This is particularly true of such foodstuffs as asparagus and spinach and other strongly alkaline and delicately flavored food- 20 stuffs, increasing the two-way reaction and being more deleteriously affected by the resultant transfer of odor and taste, causing a decided contamination of taste. In fact, no suitable lining for 25 these two foodstuffs has hitherto been developed or employed, even though zinc oxide has been incorporated in the lining composition.

I have discovered that two-way reactions through an oleoresinous film may be inhibited and largely prevented by incorporating in the 30 film overlapping plate-like particles of a chemically inert substance. The inhibiting of two-way reaction through the film appears to be the result of the screening action of the overlapping plate-like particles. My invention, based on this 35 discovery, provides an inexpensive metal food container in which black-etch is eliminated and contamination of taste is reduced to a minimum.

A food container embodying my invention comprises a metal receptacle such as a tin can having 40 on its inner surface a film incorporating a sub-stantial amount of overlapping plate-like par-ticles of a chemically inert substance. Most sat-isfactory results have been obtained by incor-porating in the dried film approximately 20% by 45 weight of plate-like particles of mica (magnesium aluminum silicate).

In making such a food container, I incorporate the mica in an oleoresinous varnish containing 50 a minor proportion of zinc oxide such as has heretofore been used for coating metal food containers, and then apply the varnish to the inner surface of a metal receptacle or to one surface of a piece of sheet metal from which the receptacle 55 may be formed. While any type of oleoresinous varnish heretofore used for food containers may be used, I prefer to incorporate the mica in a varnish which is set by baking. Such a varnish may consist of a phenol formaldehyde resin and 60 a drying oil such as tung oil. While the propor-

tion of mica in the varnish is most desirably about 10% by weight, it may be varied from not less than 5% to not more than 15%.

The following is a specific example of my composition in which zinc oxide is incorporated for 5 alkaline foodstuffs, including asparagus and spinach:

## Example No. 1

|                                          |          |
|------------------------------------------|----------|
| Modified phenol-formaldehyde resin (Par- | 10       |
| anol) -----                              | 16.55    |
| Tung oil -----                           | 24.96    |
| Linseed oil -----                        | 2.10     |
| Kerosene (Rayolite) -----                | 8.35     |
| Coal tar naptha (Hi Flash naptha) -----  | 9.85     |
| Petroleum naptha (Varnolene) -----       | 15 26.35 |
| Mica -----                               | 9.34     |
| Zinc oxide -----                         | 2.50     |
|                                          | 100.00   |
|                                          | 20       |

The following example illustrates my composition for fruits and acid foodstuff when zinc oxide is not employed:

## Example No. 2

|                                          |          |
|------------------------------------------|----------|
| Modified phenol-formaldehyde resin (Par- | 25       |
| anol) -----                              | 19.25    |
| Tung oil -----                           | 30.50    |
| Kerosene (Rayolite) -----                | 10.00    |
| Petroleum naptha (Varnolene) -----       | 22.38    |
| Coal tar naptha (Hi Flash naptha) -----  | 30 11.40 |
| Mica -----                               | 6.47     |
|                                          | 100.00   |

What I claim is:

1. A food container consisting of a metal receptacle and a film on the inner surface of said receptacle incorporating overlapping plate-like particles of mica which inhibit two-way reactions through the film.

2. A container for alkaline foodstuffs consisting of a metal receptacle and an oleoresinous film containing a minor proportion of zinc oxide on the inner surface of said receptacle incorporating overlapping plate-like particles of mica which inhibit two-way reactions through the oleoresinous film.

3. A container for alkaline foodstuffs comprising a metal receptacle and an oleoresinous film containing a minor proportion of zinc oxide on the inner surface of said receptacle incorporating from 10% to 25% by weight of plate-like particles of mica.

4. A container for alkaline foodstuffs comprising a metal receptacle and an oleoresinous film containing a minor proportion of zinc oxide on the inner surface of said receptacle incorporating approximately 20% by weight of plate-like particles of mica.